

# UNITED STATES PATENT OFFICE.

HARRY B. CHALMERS, OF QUOGUE, NEW YORK, ASSIGNOR TO LAWRENCE B. DUNHAM, OF NEW YORK, N. Y.

## PAINT AND VARNISH REMOVER.

1,079,635.

Specification of Letters Patent.

Patented Nov. 25, 1913.

No Drawing.

Application filed October 18, 1911. Serial No. 655,374.

To all whom it may concern:

Be it known that I, HARRY B. CHALMERS, a citizen of the United States of America, and a resident of Quogue, county of Suffolk, and 5 State of New York, have invented certain new and useful Improvements in Paint and Varnish Removers, of which the following is a specification.

My invention relates to improvements in 10 detergents and its object is to bring into solution with a third body, a petroleum product and an alcoholic body which are not miscible with each other. This is highly desirable in the arts but so far as I am 15 aware, has not hitherto been accomplished.

The invention is particularly useful in paint and varnish removers.

As is commonly known petroleum products such as commercial gasolene, will not 20 mix with alcoholic bodies such as ordinary wood alcohol, but I have discovered that both of these substances are simultaneously miscible with a small amount of oleic acid, and in fact the addition of a small percent- 25 age of oleic acid forms a solution of many of the light petroleum products, with methyl or ethyl alcohols, esters, or with acetone.

As an example or illustration of one of the forms of my invention and a mixture 30 which I have found useful, the following ingredients may be specified: 47 $\frac{1}{2}$  parts commercial gasolene, 15 parts of oleic acid double-pressed, 50 parts of 97% wood alcohol in which mixture 2 $\frac{1}{2}$  parts of paraffin and cer- 35 esin wax may be held in solution. The two waxes are first melted together and are preferably introduced into the liquid mixture herein described, while they are hot.

Obviously my invention and discovery is 40 capable of wide variations without departing from the scope thereof, and there are doubtless many advantageous uses for it other than those which I have as yet thought of. One of the uses is as a cleaning com- 45 pound.

The gasolene is a solvent of the waxes, but the alcohol is not. The gasolene has some detergent action on various kinds of matter, and the alcohol has a stronger solvent action 50 thereon. The gasolene and alcohol are not miscible. Neither is a gasolene solution of the waxy body miscible with the alcohol. If either the gasolene and alcohol are put together, or, a gasolene solution of the waxy

body and the alcohol are put together, an 55 immiscible volume, comparable to oil and water, so far as concerns immiscibility, results. It is not the addition of any and all proportions of oleic acid that results in effecting an approximately stable mixture of 60 the gasolene, wax and alcohol, but the addition of not substantially less than fifteen parts of oleic acid, as mentioned in the above formula. If less than fifteen per cent. of 65 oleic acid is added, the volume still remains immiscible. On addition of about fifteen per cent. of oleic acid, however, the there- 70 fore immiscible volume of gasolene, methyl alcohol and wax becomes dissolved and pulpified to about the consistency of applesauce, for example. The solution thus obtained is not, however, perfectly stable, for at most temperatures some of the gasolene floats in the upper part of the pulpified mass; and the detergent is best shaken be- 75 fore using. A further peculiarity of my new detergent lies in the fact that although it contains a wax, a wax-solvent, and an al- 80 cohol, yet it does not, when applied to sur- faces, in exposure to air, skin over or form a glassy pellicle, which is a characteristic of some detergents containing a wax-solvent like benzol, which is immiscible with alcohol, a waxy body and alcohol but without the addition of oleic acid. This acid, which 85 I use, has some peculiar property in pulp- 90 ifying the wax, the wax-solvent and the al- cohol, if about fifteen per cent. or more of oleic acid is used. If a much larger per- 95 centage is used, the detergent is unduly weakened. On the other hand, if approxi- 100 mately fifteen per cent. of oleic acid is not used, no pulpifying action results.

One marked advantage of this invention is that it discloses a hitherto unknown mode 95 of utilizing in an alcoholic wax containing detergent, a wax-solvent that is immiscible with alcohol. A further advantage of this detergent is that as it does not skin over or form a glassy pellicle in use, it cannot, if allowed to remain in place, form an additional, more or less solid coat, on a painted or varnished surface, for example, to which it may be applied.

What I claim is:

1. A detergent comprising approximately 105 equal parts of gasolene and alcohol with ap- proximately fifteen per cent. of oleic acid,

the same forming a pulpified mass which is characterized by not skinning over on exposure to the atmosphere.

2. A detergent of pulpified consistency comprising forty-seven and one-half parts of gasolene, fifty parts of ninety-per cent. wood alcohol, two and one-half parts of wax comprising half each of paraffin and ceresin wax, and fifteen parts of double-pressed oleic acid; the latter acting to pulpify the

immiscible volume of the gasolene, wood alcohol and wax.

In witness whereof, I have hereunto set my hand this 13th day of October, 1911, in the presence of two witnesses.

HARRY B. CHALMERS.

Witnesses:

ERNEST W. MARSHALL,  
F. GRAVES.